

June 17, 1941.

E. O. NORRIS

2,246,380

ELECTROLYTIC METHOD OF PRODUCING SCREENS

Filed Feb. 19, 1938

3 Sheets-Sheet 1



INVENTOR  
EDWARD O. NORRIS

BY  
John H. Willard  
ATTORNEY

June 17, 1941.

E. O. NORRIS

2,246,380

ELECTROLYTIC METHOD OF PRODUCING SCREENS

Filed Feb. 19, 1938

3 Sheets-Sheet 2



*Fig. 2.*



*Fig. 3.*



*Fig. 4.*

INVENTOR  
EDWARD O. NORRIS

BY

*John H. Willard*  
ATTORNEY

June 17, 1941.

E. O. NORRIS

2,246,380

ELECTROLYTIC METHOD OF PRODUCING SCREENS

Filed Feb. 19, 1938

3 Sheets-Sheet 3

*Fig. 8.*



*Fig. 9.*



*Fig. 10.*



INVENTOR  
EDWARD O. NORRIS.

BY  
*John H. Billiard*  
ATTORNEY

## UNITED STATES PATENT OFFICE

2,246,380

ELECTROLYTIC METHOD OF PRODUCING  
SCREENS

Edward O. Norris, Westport, Conn., assignor to  
Edward O. Norris, Inc., New York, N. Y., a corporation of New York

Application February 19, 1938, Serial No. 191,405

5 Claims. (CL 204—11)

This application contains matter taken from my application Ser. No. 138,301, filed April 22, 1937, and is a continuation in part thereof.

The present invention has for an object to provide a metallic screen having reinforcements integrally united therewith and also to provide a process for the manufacture of such screens or for applying such reinforcements to existing screens.

My process is particularly adapted for the production or reinforcement of fine mesh screens, although it is not limited thereto but may be applied to advantage in the manufacture of screens of relatively coarse mesh, since the product combines strength and a desired degree of rigidity with lightness and economy due to the reduction in weight of metal used.

In the manufacture of fine mesh sheet metal screens formed by electrolytic deposition of metal, where there are practical limits to the thickness of metal that can be deposited without closing up the apertures, my process is of special value as a means of adding requisite strength to the screen.

In my co-pending application Serial No. 52,334, filed November 30, 1935, now Patent No. 2,166,366, I describe a matrix comprising a metallic plate formed with a pitted surface, the pits being filled with insulating material to the level of said surface, thus masking or electrically blanking out dots thereon, so that when metal is deposited electrolytically on the matrix it will form a sheet with an aperture therein at each dot. It is found, however, that as the electrolytic process continues the metal tends to grow over the spots of insulation, and if the process is continued long enough, the metal will close the apertures completely. It will be obvious, therefore, that with such a matrix the mesh of the screen imposes limits upon the thickness of metal that may be deposited, for, as the sheet grows thicker, the apertures grow smaller and, obviously, the spacing of the apertures grows greater. In the case of very fine screens the sheet may be too fragile or flimsy for practical use, and my reinforcing process is particularly adapted to give desired strength to such fine mesh screens.

A more specific object of my invention is to form a fine mesh screen in the manner described above and then to reinforce said screen with a relatively coarse mesh screen formed by electrolytic deposition of metal on the fine mesh screen. Each mesh of the coarse screen then provides a reinforcing frame for a limited area of the fine screen. In other words, the resultant

product may be considered as a sheet of metal formed with pockets each having a finely perforated floor. With this structure it is possible to produce screens in which the apertures are of microscopic dimensions and yet in which the screen as a whole is of substantial strength.

While I prefer to apply the reinforcement in the form of a relatively coarse screen or grid, it is within the purview of my invention to apply the reinforcement in parallel non-intersecting ribs, or, in any other desired pattern. The reinforcement may be applied to one face only of the screen leaving the opposite face smooth, or, if desired, the reinforcing ribs may project from each surface of the screen.

Other objects and advantages of my invention will appear in the following description of certain forms of reinforced screens and processes of forming the same, and thereafter the novelty and scope of the invention will be pointed out in the claims.

In the accompanying drawings:

Fig. 1 is a view in perspective of part of a matrix on which the initial fine mesh screen is to be formed;

Fig. 2 is a similar view showing a fine mesh screen formed on the matrix by electrolytic deposition of metal;

Fig. 3 is a view in cross-section illustrating a further step of the process wherein a grid or coarse mesh screen is formed on the fine mesh screen;

Fig. 4 is a view in cross-section of the finished screen;

Fig. 5 and Fig. 6 illustrate certain steps of a modified process, Fig. 5 being a view in perspective illustrating one of the steps, and Fig. 6 a view in cross-section illustrating another step in the process;

Fig. 7 is a view in cross-section of the screen produced by such modified process;

Figs. 8 and 9 illustrate certain steps of another modification of the process, Fig. 8 being a view in perspective of part of a specially prepared matrix and Fig. 9 being a view in cross-section showing the reinforced screen formed on said matrix; and

Fig. 10 is a view in cross-section of a screen produced by the process illustrated in Figs. 8 and 9.

The matrix, shown in Fig. 1, comprises a metallic plate 12 formed with depressions to receive inserts 13 of a material that is an insulator of electricity. The exposed faces 14 of these inserts are flush with the upper face of the plate 12

and are separated by intersecting lanes 15 of conducting material constituting the exposed metallic surface of the plate 12. The present application is not concerned with the manufacture of the matrix which may be formed in the manner described in said copending application Serial Number 52,334. It will be understood, of course, that in actual practice the areas 14 need not necessarily be square nor so uniformly contoured, as shown in Fig. 1. Actually the areas 14 may be of microscopic dimensions and spacing.

The matrix 12 is suitably treated and used as the cathode in an electro-plating bath, whereby metal will be deposited upon the exposed metallic lanes 15 but not on the surfaces 14. Thus, a screen will be built up on the matrix, as shown in Fig. 2, composed of intersecting ribs 16 overlying the lanes 15. The electro-deposition is continued until a predetermined thickness of metal is formed, but, as clearly shown in Fig. 2, the deposited metal will form ribs of semi-cylindrical cross-section which, as they grow, must necessarily overlap the surfaces 14, and the reduction in size of the apertures in the screen imposes a limit on the thickness of metal that may be deposited.

The next step in the process consists in blanking out areas of the fine screen by printing or otherwise applying thereon spots of ink or other non-conducting material, as indicated at 18 in Fig. 3. Each spot 18 covers a large number of the apertures in the fine screen and the spots are separated by bare spaces exposing the metal surface of the screen. These spaces are preferably in the form of intersecting lanes much broader and much more widely spaced than the lanes 15. The screen thus treated and still on its matrix is again placed in an electroplating bath, and metal is again deposited, this time forming only in the exposed lanes between the flanged out portions 18. The electro-deposition may be continued to such an extent as to build up relatively heavy ribs 19 of sufficient cross-section to provide the desired reinforcement to the screen. The final step in the process is to wash off the ink or coating material 18 and strip the product from the matrix. The resultant reinforced screen will then appear as shown in Fig. 4, comprising a coarse screen portion formed of intersecting ribs 19 integrally united to the fine mesh screen portion formed of the intersecting ribs 16.

In applying the reinforcement to the fine mesh screen I prefer to maintain the screen on the matrix. However, it will be obvious that the screen may be stripped from the matrix before the reinforcement is applied. In such case, one face of the screen may be completely blanked out, or both faces may have insulation areas 18 printed thereon, so that reinforcing ribs 19 will be formed on each face of the fine mesh screen.

If it be desired to form a screen with a heavier reinforcing the modified process illustrated in Figs. 5 and 6 may be employed. In this modified process, after forming the original fine mesh screen, as shown in Fig. 2, a layer 20 of a different metal is electrolytically deposited upon the screen, as shown in Fig. 5. After the layer 20 has been deposited upon the screen to desired thickness, the surface thereof is printed or otherwise coated with spots 21 of a suitable resist material, leaving intervening bare spaces exposing the metallic surface of layer 20. Each spot 21 covers a relatively broad area sufficient to embrace a large number of apertures of the fine mesh screen. The product thus prepared is then

placed in an electro-plating bath and metal is deposited on the exposed areas, building up ribs 22.

The next step of the process consists in removing the resist to expose the layer 20 so that it may be eaten away by a suitable etching fluid. The ribs 22 as well as the ribs 16 must be formed of a metal that is either immune to attack by said etching fluid or offers high resistance thereto. For instance, the ribs 16 and 22 may be formed of nickel and the layer 20 of copper. Suitable etching reagents for etching out the copper layer are (1) a solution of potassium cyanide or (2) a mixture of chromic and sulphuric acids in water, suitable proportions being about as follows:

|                |   |         |    |
|----------------|---|---------|----|
| Sulphuric acid | — | pounds  | 2  |
| Chromic acid   | — | do      | 1  |
| Water          | — | gallons | 10 |

Neither of these reagents will have any appreciable effect on the nickel during the comparatively brief time required for etching the copper. However, such portions of the copper layer as are covered by ribs 22 will be protected from the etching fluid at least to the extent that they will form connecting webs 23 between ribs 22 and the fine mesh screen. Thus, as shown in Fig. 7, the final product will be a composite screen comprising the initial fine mesh reinforced by a coarse mesh integrally united thereto by the copper webs 23.

Instead of eating out the copper with an etching fluid it may be removed by deplating or electro-etching. In other words, the work is connected up as the anode in a suitable electroplating bath and the copper that is not protected by the overlying nickel ribs is then removed electrolytically.

Another method of producing a reinforced fine mesh screen is shown in Figs. 8 and 9. In this case, the deposit receiving surface of the matrix 12 is machined to form grooves 25 therein, which intersect preferably at right angles to each other, so as to leave islands 26 therebetween. Each island surface consists of a portion of the original matrix surface, comprising exposed metal lanes 15 and insulated surfaces 14. The grooves 25 are cut to a depth well below that of the inserts 13.

The matrix thus prepared is now placed in an electroplating bath and metal is deposited on the lanes 15, to form the ribs 16. The electro-plating is stopped when the apertures between the ribs are reduced to a predetermined extent by overlap of the deposited metal on the insulated areas 14. This metal is also deposited in the grooves 25, forming channel-shaped walls 27 running lengthwise and transversely of the screen. Upon the screen thus produced a metal layer 28 is then deposited. This metal completely covers the original screen and also forms depressed webs 29 in the channel-shaped portions 26. The surface of layer 28 is then printed or coated with a suitable resist, as indicated at 30. This coating is interrupted by the depressed webs 29 which are left bare.

The next step of the process consists in placing the web in another electro-plating bath to form a third deposit of metal thereon. This metal will form only on the webs 29, and the deposition of metal is continued until the channel-shaped webs are completely filled and the metal has been built up to a desired height above layer 28, thus forming a grid or coarse screen composed of ribs 31. The layer 28 is formed of metal

which is soluble in an etching fluid that has little or no effect on the metal of ribs 16 and ribs 31, or which may be depleted without appreciable effect on said ribs. Preferably, the layer 28 is formed of copper, while the ribs 16, channels 27, and ribs 31, may be made of nickel.

The final step of the process consists in washing off the insulation 30 and removing the copper layer 28 either with an etching reagent, such as has been already mentioned, or by deplating. Part of the webs 29 will be protected by the overlying ribs 31 and will provide means anchoring said ribs in the channels 27. The work is then stripped from the matrix, producing a finished screen, such as shown in Fig. 10. This, it will be seen, consists of the original fine mesh screen reinforced by a coarse mesh screen composed of the ribs 30. This reinforcement projects below as well as above the plane of the ribs 16 which form the fine mesh screen.

In the following claims the word "etching" is used in its broad sense to include the removal of metal either by electro-etching or by fluids which attack the metal without the aid of electric current.

I have described above certain embodiments of my invention and a preferred process with certain modifications thereof, but I wish it to be understood that these are illustrative and not limitative of my invention and that I reserve the right to make various changes in form, construction and arrangement of parts and also to make various changes in process of manufacture falling within the spirit and scope of my invention, as set forth in the claims.

I claim:

1. A process of reinforcing a thin metallic screen, which comprises the steps of electro-depositing on the screen a layer of metal that may be selectively etched to the exclusion of the metal of the screen, blanking out spaced areas of said layer with electric insulation material but leaving intersecting lanes of bare metal between said areas, electro-depositing in said lanes ribs of a metal resistant to an etching reagent that reacts on the metal of the said layer, removing said insulation material, and etching out all of said layer except narrow web portions integrally connecting said ribs to the screen by means of an etching reagent that reacts on the metal of the said layer but does not react on the material of the screen or the material of said ribs.

2. A process of making a reinforced metallic screen, which comprises the steps of electro-depositing metal on the surface of a matrix dotted with electric insulation and thereby forming a thin, finely apertured, metal sheet, electro-depositing on said sheet a layer of metal reactive to an etching reagent that does not react on the material of said screen, blanking out spaced areas

5 of said layer with electric insulation but leaving intersecting lanes of bare metal between said areas, electro-depositing metal resistant to an etching reagent that acts corrodably on the material of said layer, removing said insulation, etching out all of said layer except narrow portions thereof protected by the metal in said lanes by means of an etching reagent that acts corrodably on the metal of said layer but is substantially inert with respect to the metal of said screen and the metal deposited in said lanes, and stripping the screen from the matrix.

3. A process of making a reinforced metallic screen, which comprises the steps of electro-depositing nickel on the surface of a matrix dotted with electric insulation and thereby forming a finely apertured nickel sheet, electro-depositing a layer of copper on said sheet, blanking out areas of said layer with electric insulation but 10 leaving intersecting lanes of the bare metal between said areas, electro-depositing nickel in said lanes to build up a reinforcement grid, removing said insulation, and etching the copper layer with an etching reagent that selectively etches copper to the exclusion of nickel, thereby removing all of said layer except narrow web portions connecting said grid to said sheet.

4. A process of making a metallic screen, which comprises the steps of preparing a metallic matrix with a plurality of electrically insulated dots on a surface thereof, grooving said surface to form a plurality of spaced lands, each land including a multiplicity of said dots, electro-depositing metal on said surface to form a thin metallic sheet with apertures therein at said dots, 15 protecting the outer surface of the sheet over each of said lands, electro-depositing metal between said lands and thereby forming ribs within said grooves integrally connected to said metallic sheet, and stripping the sheet from the matrix.

5. A process of making a reinforced metallic screen, which comprises the steps of forming a metallic matrix having a surface thereof dotted with electric insulation material, grooving said surface to form isolated lands, each land including a multiplicity of such insulation dots, electro-depositing nickel on the matrix to produce a thin nickel sheet with apertures therein at said dots and with channel webs formed in said grooves, electro-depositing a layer of copper on said apertured sheet and said channel webs, applying a coating of electric insulation on said layer over said lands but not over said channel webs, electro-depositing nickel ribs on the copper layer over the channel webs, removing said insulation, and etching to remove all of the copper except narrow portions thereof connecting the ribs to said sheet.

EDWARD O. NORRIS.